

## United States Patent [19]

Idota et al.

[11] 4,301,236

[45] Nov. 17, 1981

## [54] PHOTOGRAPHIC BLEACH SOLUTIONS

[75] Inventors: Yoshio Idota; Minoru Yamada, both of Minami-ashigara, Japan

[73] Assignee: Fuji Photo Film Co., Ltd., Kanagawa, Japan

[21] Appl. No.: 114,456

[22] Filed: Jan. 23, 1980

## [30] Foreign Application Priority Data

Jan. 23, 1979 [JP] Japan ..... 54-6645

[51] Int. Cl. 3 ..... G03C 5/32

[52] U.S. Cl. ..... 430/393; 430/430; 430/461; 430/943; 252/95; 252/99; 252/102

[58] Field of Search ..... 430/393, 430, 461, 943; 252/102, 95, 99

[56]

## References Cited

## U.S. PATENT DOCUMENTS

|           |         |                       |         |
|-----------|---------|-----------------------|---------|
| 3,532,634 | 10/1970 | Woods .....           | 252/95  |
| 3,820,997 | 6/1974  | Shirasu et al. ....   | 430/393 |
| 3,870,520 | 3/1975  | Shimamura et al. .... | 430/393 |
| 4,119,557 | 10/1978 | Postlethwaite .....   | 252/95  |
| 4,203,765 | 5/1980  | Claeys et al. ....    | 430/430 |

*Primary Examiner*—J. Travis Brown*Attorney, Agent, or Firm*—Sughrue, Mion, Zinn, Macpeak & Seas

[57]

## ABSTRACT

A bleach solution for color photographic materials having a high bleaching activity and capable of providing color images having good quality containing hydrogen peroxide or a compound releasing hydrogen peroxide, an organic metal complex salt, and an unsubstituted or substituted aromatic sulfonic acid or a salt thereof.

23 Claims, No Drawings

## PHOTOGRAPHIC BLEACH SOLUTIONS

## BACKGROUND OF THE INVENTION

## 1. Field of the Invention

This invention relates to a photographic processing for silver halide color photographic materials and, more particularly, to a photographic bleach solution for silver halide color photographic materials having a sufficient bleaching activity and capable of forming color images having good quality.

## 2. Description of the Prior Art

In photographic processing for silver halide color photographic materials, a color photographic material (the silver halide photographic emulsions thereof may have been fogged beforehand) is developed in an ordinary manner, after being imagewise exposed using a developer containing an aromatic primary amine color developing agent in the presence of dye forming couplers to provide color images and developed silver formed simultaneously with the formation of the color images is re-halogenated by bleaching and is removed by fixing (or blixing) together with undeveloped silver halides.

Hitherto, a ferricyanide, ferric chloride, aminopolycarboxylic acid ferric complex salt, etc., have mainly been used as a bleaching agent. A ferricyanide and ferric chloride are good bleaching agents in the points that they have a sufficiently high bleaching speed (oxidizing speed) and developed silver is sufficiently oxidized in a definite period of time. However, since a bleach solution using a ferricyanide as bleaching agent liberates a cyan ion by photodecomposition to cause environmental pollution, a treatment must be applied to make the waste bleach solution completely nontoxic. Also, a bleach solution using ferric chloride as bleaching agent has a fault that parts of a processor containing the bleach solution are liable to be corroded owing to the very low pH and very large oxidative power as well as has a fault that in the wash step after bleach processing, iron hydroxide deposits in silver halide emulsion layers to cause so-called stains. Consequently, a cleaning step by an organic chelating agent must be applied after bleaching, which conflicts with the purposes to process quickly and save labour, and also the use of such a bleach solution is undesirable in terms of environmental problems since there is a danger of generating a hydrogen chloride gas.

On the other hand, a metal complex of an organic acid such as a metal complex salt of aminopolycarboxylic acid gives less environmental pollution as compared with a ferricyanide or ferric chloride and hence such a complex salt has frequently been used recently as bleaching agent. However, an organic metal complex as bleaching agent has generally a relatively low oxidative power and is also insufficient in bleaching power, when a bleaching solution using the complex salt as bleaching agent is used for bleaching, for example, a desired object may be attained to some extent using low speed silver halide color photographic materials mainly composed of silver chlorobromide emulsions, but when the bleach solution is used for bleaching high speed silver halide color photographic materials which are mainly composed of silver iodochlorobromide emulsions or silver iodobromide emulsions and have been color-sensitized, (in particular silver halide color photographic materials using high silver content silver halide emulsions) the removal of silver becomes poor due to the

insufficient bleaching action and so-called poor recoloring occurs (i.e., the dyes formed by the oxidative coupling of the oxidation product of a color developing agent and couplers remain as leuco dyes which are reaction intermediates). The term "high silver content silver halide emulsions" as used herein refers to silver halide emulsions having no more than 30-40 mg/100 cm<sup>2</sup> of the total silver amount in blue-sensitive, green-sensitive and red-sensitive silver halide emulsion layers.

Thus, to rapid processing high speed silver halide color photographic materials it is necessary to overcome these difficulties.

As a process for overcoming the difficulties, it is proposed in Japanese patent application (OPI) No. 109731/75 (The term "OPI" as used herein refers to a "published unexamined Japanese patent application") to use an iron or cobalt complex salt of an organic acid together with hydrogen peroxide. In general, in the case of using such a bleach solution, leuco compounds are effectively converted into dyes immediately after the preparation of the bleach solution but it has a fatal fault that when the bleach solution is allowed to stand after the preparation thereof, the oxidative power thereof rapidly decreases and the oxidation of silver and the oxidation of leuco compounds become insufficient. This fault exists even in a range of acidic side (pH 2-6) at which the bleach solution is said to be relatively stable. This is considered to be caused by the acceleration of the decomposition of hydrogen peroxide by metal ions.

Furthermore, the use of hydrogen peroxide is accompanied by a fault that the layers of photographic materials are broken during processing. Also, a metal such as stainless steel, etc., is used for automatic processors and in case of using such a bleach solution, there is a fault that hydrogen peroxide contained in the bleach solution causes self-decomposition by the catalytic action of the metal to reduce the bleaching power of the bleach solution.

Moreover, even in the case of aminopolycarboxylic acid iron complexes, when the complexes are used in large quantities, the concentration of iron ions increases, which is undesirable for environmental reasons.

On the other hand, since hydrogen peroxide forms water by the decomposition, it is an ideal oxidizing agent which causes no environmental pollution. Therefore, it has long been desired in this field of art to use practically a bleach solution for color photographic materials using hydrogen peroxide.

However, hydrogen peroxide is a strong oxidizing agent but when hydrogen peroxide is simply used as a bleaching agent, it is impossible to practically use hydrogen peroxide for bleaching silver in color photographic materials.

## SUMMARY OF THE INVENTION

A first object of this invention is, therefore, to provide an effective bleach solution for silver halide color photographic materials containing hydrogen peroxide as the main bleaching component.

A second object of this invention is to provide a bleach solution of silver halide color photographic materials causing no environmental pollution, having excellent storage stability, and showing a high bleaching speed.

A third object of this invention is to provide a processing process for silver halide color photographic materials without so-called poor recoloring phenome-

non that the dyes formed by oxidative coupling remain in the state of leuco dyes after bleach step.

A fourth object of this invention is to provide a process for processing silver halide color photographic materials which always maintains a stable bleaching power.

The objects of this invention can be attained by a bleach solution comprising hydrogen peroxide (or a compound releasing hydrogen peroxide or a mixture of hydrogen peroxide and a compound releasing hydrogen peroxide), an organic acid metal complex salt, and at least one substituted or unsubstituted aromatic sulfonic acids (including salts thereof and the acid may have two or more sulfon groups).

#### DESCRIPTION OF THE INVENTION

The organic acid metal complex salts used in this invention are compounds having the ability to convert metallic silver formed by development into silver halide by oxidizing it and simultaneously converting leuco dyes into dyes, and they have a structure formed by chelating an aminopolycarboxylic acid, an organic phosphonic acid, or polycarboxylic acid such as citric acid, oxalic acid, etc., with a high valent metal ion such as iron (III) ion, cobalt(III) ion, copper(II) ion, etc. Chelating agents used for forming the complex salts used in this invention are the polycarboxylic acids represented by following formula I:



(I) 30

wherein  $R_1$  represents a single bond, an unsubstituted or substituted alkylene group having 1 to 6 carbon atoms wherein the substituent is a hydroxy group and/or a carboxy group, a  $-(CH_2)_m-O-(CH_2)_n-$  group wherein  $m$  and  $n$  are integers and  $m+n$  is 2 to 6, a  $-(CH_2)_m-S-(CH_2)_n-$  group wherein  $m'$  and  $n'$  are integers and  $m'+n'$  is 2 to 6, or an alkenylene group having 2 to 6 carbon atoms;  $l$  represents an integer of 2 to 3; and when  $R_1$  is a single bond,  $l$  is 2.

Typical examples of the polycarboxylic acid represented by the formula (I) are as follows:

Citric acid,  
Oxalic acid,  
Malonic acid  
Tartaric acid,  
Diglycolic acid, and  
Thiodiglycolic acid.

Chelating agents used for forming the complex salts used in this invention are the aminopolycarboxylic acids represented by following formula II:



(II)

55

wherein  $R_2$ ,  $R_3$ ,  $R_4$  and  $R_5$  each represents a carboxyalkyl group wherein the alkyl moiety has 1 to 2 carbon atoms, a hydroxyalkyl group having 1 to 2 carbon atoms and/or a hydrogen atom;  $p$  represents zero or an integer of 1 to 3;  $L$  represents an alkylene group having 2 to 4 carbon atoms, a  $-(CH_2)_x-O-(CH_2)_y-$  group wherein  $x$  is an integer of 2 to 4,  $y$  is an integer of 2 to 4 and  $z$  is an integer of 1 to 3, a 6-membered cyclic alkylene group, or an arylene group (e.g., phenylene); and the aminopolycarboxylic acid of the formula (II) has at least 1 carboxy group.

Typical examples of the aminopolycarboxylic acids of the formula (II) or the salts thereof are as follows:

Ethylenediaminetetraacetic acid,  
Ethylenediaminetetraacetic acid disodium salt,  
Ethylenediaminetetraacetic acid diammonium salt,  
Ethylenediaminetetraacetic acid tetra(trimethylammonium) salt,  
Ethylenediaminetetraacetic acid tetrapotassium salt,  
Ethylenediaminetetraacetic acid tetrasodium salt,  
Ethylenediaminetetraacetic acid trisodium salt,  
Diethylenetriaminepentaacetic acid,  
Diethylenetriaminepentaacetic acid pentasodium salt,  
Ethylenediamine-N-( $\beta$ -oxyethyl)-N,N',N'-triacetic acid,  
Ethylenediamine-N-( $\beta$ -oxyethyl)-N,N',N'-triacetic acid sodium salt,  
Ethylenediamine-N-( $\beta$ -oxyethyl)-N,N',N'-triacetic acid triammonium salt,  
Propylenediaminetetraacetic acid,  
Propylenediaminetetraacetic acid sodium salt,  
Nitrilotriacetic acid,  
Nitrilotriacetic acid sodium salt,  
Cyclohexanediaminetetraacetic acid,  
Cyclohexanediaminetetraacetic acid sodium salt,  
Iminodiacetic acid,  
Dihydroxyethylglycine,  
Ethyl ether diaminetetraacetic acid,  
Glycol ether diaminetetraacetic acid,  
Ethylenediaminetetrapropionic acid, and  
Phenylenediaminetetraacetic acid.

Chelating agents used for forming the complex salts used in this invention are the organic phosphonic acids represented by following formulae III-a or III-b:



wherein  $R_6$  represents a substituted or unsubstituted alkyl or alkylene group having 1 to 4 carbon atoms wherein the substituent is a hydroxy group and/or a carboxy group, or a substituted or unsubstituted diaminoalkylene group having 2 to 16 carbon atoms wherein the substituent is a hydroxy group;  $L$  represents an alkylene group having 1 to 2 carbon atoms; and  $q$  represents an integer of 1 to 5.

Typical examples of the organic phosphonic acids of the formulae III-a and III-b are as follows:



Although the invention is not limited to the compounds thus illustrated above.

Preferred examples of the chelating agent are an ethylenediaminetetraacetic acid and a salt thereof and an ethylenediamine-N-( $\beta$ -oxyethyl)-N,N'-N'-triacetic acid and a salt thereof.

As the metal ions, ferric ions are preferred and in this case, the proportion of the ferric ions is 0.0001 to 2 moles, preferably 0.01 to 0.2 mole per liter of bleach solution. 30

As compounds releasing hydrogen peroxide used in this invention, perboric acid (or salts thereof), and per-carbonic acid (or salts thereof) are preferred. Urea-hydrogen peroxide compound and peracetic acid are also useful. The proportion of hydrogen peroxide or the compound releasing hydrogen peroxide is about 0.1 to 10 moles, preferably 0.1 to 2 moles per liter of bleach solution. In this invention, a preferred effect is achieved if the mole number of hydrogen peroxide (or precursor) per liter of the bleach solution is larger than that of the ferric ion and further it is more preferred that the mole number of the hydrogen peroxide is twice as large as the ferric ion. 35 40 45 46

The substituted or unsubstituted aromatic sulfonic acids (or salts thereof) or substituted or unsubstituted aromatic polyvalent sulfonic acids (or salts thereof) 50 used in this invention can be represented by following formula IV:



wherein M represents a hydrogen atom, an alkali metal atom (e.g., sodium or potassium), or an ammonium group; r represents an integer of 1 to 5; and Q represents an aromatic hydrocarbon group or an aromatic heterocyclic group including at least one nitrogen atom or sulfur atom. These aromatic groups may have one or more substituents. Examples of the substituents are aliphatic groups or aromatic hydrocarbon groups (each of which may be substituted by, e.g., a carboxyl group, a hydroxy group, an amino group, a nitro group, a nitroso group, or a halogen atom), a carboxy group, a hydroxy group, an amino group, a nitro group, a nitroso group, and a halogen atom. 55 60 65

Practical examples of the compounds represented by general formula IV are illustrated below:



A proper addition amount of the compound shown by general formula IV is about  $5 \times 10^{-5}$  to 0.3 mole,

preferably about  $10^{-3}$  to 0.1 mole per liter of bleach solution. In the case of polymer, it means a mole number of sulfon groups.

This invention is distinguished from conventional techniques by the following reasons.

Hydrogen peroxide itself has very low rate for oxidizing silver but when a very small amount of a ferric ion which oxidizes silver very slowly is added to hydrogen peroxide, the rate of bleaching silver by the system becomes very high. Thus, it is expected that hydrogen peroxide is decomposed by the catalytic action of the iron ions to generate an oxidative power (this is well known decomposition reaction of a Fenton reagent). On the other hand, Japanese patent application (OPI) No. 102296/78 discloses that a condensation product of naphthalenesulfonic acid and formalin controls the decomposition of hydrogen peroxide in the presence of iron ions. Therefore, in spite of the expectation that the addition of a compound having a sulfon group will be accompanied by a side-action, i.e., a reduction in bleaching rate, on the contrary, the bleaching rate is not reduced by the addition of a compound having a sulfon group and further the reduction in oxidative power during storage as occurs in the above-described co-existing system of ferric ions and hydrogen peroxide can be prevented, and hence the invention provides an effect which is unusual by comparison to the conventional techniques.

In this invention, a ferric ion exists at the above-described concentration and the existence of the ion has the effect of increasing the storage stability of the bleach solution containing hydrogen peroxide as the main component.

Furthermore, the bleach solution of this invention has the following effect. That is, it is known that hydrogen peroxide causes self-decomposition by the catalytic action of a metal such as stainless steel but the bleach solution of this invention can restrain the self-decomposition of hydrogen peroxide and hence stainless steel, 40 titanium alloys, etc., can be used for automatic precursors in this invention.

The bleach solutions used in this invention may further contain various additives together with the above-described compounds.

Preferred additives used in this invention for accelerating bleaching are halides such as alkali halides and ammonium halides, for example, potassium bromide, sodium bromide, ammonium bromide, sodium chloride, etc. The addition amount of the additive is about 0.01 to 50 5 moles, preferably about 0.2 to 2 moles per liter of the bleach solution.

Furthermore, it is preferred to add an aliphatic carboxylic acid, an aliphatic phosphonic acid, or an aliphatic phosphonocarboxylic acid, such as, for example, 55 acetic acid, acetates, propionic acid, propionates, succinic acid, succinates, malonic acid, malonates, citric acid, citrates, 2,2-diphosphonoethanol or the salts thereof, and 2-phosphono-1,2,4-tricarboxylic acid or the salts thereof. The addition amount of it is about 0.01 to 5 60 moles, preferably about 0.1 to 1 mole per liter of the bleach solution.

Also, additives which are conventionally used in bleach solutions, for example, a pH buffer such as a borate, an acetate, a phosphate, etc.; a pH adjusting 65 agent such as sodium hydroxide, ammonia water, etc.; a corrosion inhibitor such as ammonium nitrate, etc.; a swelling preventing agent such as ammonium sulfate, a

surface active agent (e.g., polyethylene oxide, etc.), etc., can be properly added.

The pH of the bleach solution used in this invention is about 1 to 10, preferably about 3 to 8. The bleaching temperature is typically from 20° to 60° C.

Furthermore, in the case of processing silver halide color photographic materials using the bleach solution of this invention, a substituted alkylthiol compound or a precursor may be used as a bleach accelerator in a bath used prior to the bleach bath. Typical examples of the substituted alkylthiol compounds or the precursors thereof are described in U.S. Pat. No. 3,893,858; *Research Disclosure*, 15704 (1977, May); and Japanese patent application (OPI) Nos. 20832/77; 32736/78; 94927/78; 95630/78 and 95631/78.

The substituted alkylthiol compounds or the precursors thereof which may be used in this invention are shown by the general formula:



wherein R represents an alkyl group having 1 to 10 carbon atoms, which may have one or more substituents and may be branched; at least one of the substituents for group R being a hydroxy group, a primary, a secondary, a tertiary amino group, a carboxy group, a sulfon group, a piperidino group, a pyrrolyl group, a morpholino group, an imidazole group, or a benzotriazole group; and Y represents a hydrogen atom or an amidino group.

Practical examples of these compounds are as follows:



-continued



These compounds may form salts such as chlorides. Also, the above-described compounds are typical examples and the invention is not limited to these compounds. The addition amount of this additive is about  $1 \times 10^{-5}$  to 1 mole/liter, preferably about  $1 \times 10^{-3}$  to  $1 \times 10^{-1}$  mole/liter.

The processing baths containing these compounds include a processing bath used after the color development bath and prior to the bleach bath. For example, there is a stop bath, and a stop-fix bath.

When color photographic materials are processed using a bath containing the substituted alkylthiol compound or a precursor thereof prior to performing the bleach processing using the bleach solution of this invention, the bleaching period can be greatly shortened.

The bleach solution of this invention used can be easily reproduced for reuse by adding hydrogen peroxide thereto.

This invention can be applied to the processing of whole color photographic materials using silver halide emulsions, such as color papers, color negative films, color reversal films, color positive films, etc., but when the bleach solution of this invention is used for processing color photographic materials using high silver content silver halide emulsions having a total silver content in silver halide emulsion layers of 30 mg/100 cm<sup>2</sup> or more, the effect of this invention is large and when the invention is used for the processing of color photographic materials having a total silver amount of 40 mg or more per 100 cm<sup>2</sup>, the invention is particularly useful.

In this invention, processings for imagewise exposed color negative films, color positive films, color papers,

etc., are fundamentally composed of the following steps:

(1) color development→stop →bleach→wash→fix→wash→stabilization→dry,

(2) color development→stop→bleach→fix→wash→stabilization→dry,

(3) color development→stop→fix→bleach→fix→wash→stabilization→dry, or

(4) color development→bleach→wash→fix→wash→stabilization→dry.

In processings (1) to (4), a pre-bath, a hardening bath, etc., may be employed before the color development and also a stabilization or a wash after bleach may be omitted.

On the other hand, processings for color reversal films are fundamentally composed of the following steps:

(5) black and white development→stop→wash→fogging→wash→color development→stop→wash→bleach→wash→fix→wash→stabilization→dry or

(6) black and white development→stop→wash→fogging→wash→color development→stop→wash→bleach→fix→wash→stabilization→dry.

In processings (5) and (6), a pre-bath, a pre-hardening bath, a neutralization bath, etc., may be employed. Also, a stabilization or a wash after bleach may be omitted. Furthermore, the fogging bath may be replaced with reexposure and also by adding a fogging agent to the color developer, the fogging bath may be omitted.

In the photographic processing of this invention, the above-described steps (1) to (6) are useful but the invention is not limited to these steps.

The color developer used in this invention has a composition for ordinary color developer containing an aromatic primary amine developing agent and preferred

examples of the aromatic primary amine color developing agent are such p-phenylenediamine derivatives as N,N-diethyl-p-phenylenediamine, 2-amino-5-diethylaminotoluene, 2-amino-5-(N-ethyl-N-laurylamo)-toluene, 4-[N-ethyl-N-(β-hydroxyethyl)amino]aniline, 2-methyl-4-[N-ethyl-N-(β-hydroxyethyl)-amino]aniline, N-ethyl-N-(β-methanesulfonamidoethyl)-3-methyl-4-aminoaniline described in U.S. Pat. No. 2,193,015, N-(2-amino-5-diethylaminophenylethyl)methanesulfonamide and N,N-dimethyl-p-phenylenediamine described in U.S. Pat. No. 2,592,364, 4-amino-3-methyl-N-ethyl-N-methoxyethylaniline, 4-amino-3-methyl-N-ethyl-N-β-ethoxy-ethylaniline, 4-amino-3-methyl-N-ethyl-N-β-butoxyethylaniline, and the salts thereof

50 (e.g., sulfates, hydrochlorides, sulfites, p-toluenesulfonates, etc.), etc., described in U.S. Pat. Nos. 3,656,950; 3,698,525; etc.

The color developer may further contain other known components used in ordinary color developers.

55 For example, sodium hydroxide, potassium hydroxide, sodium carbonate, potassium carbonate, sodium or potassium tertiary phosphate, potassium metaborate, borax, etc., may be used solely or as a combination thereof as an alkaliifying agent or a buffer. Also, various salts such as di-sodium or di-potassium hydrogenphosphate, potassium or sodium dihydrogenphosphate, sodium or potassium hydrogencarbonate, boric acid, an alkali nitrate, an alkali sulfate, etc., can be also used together with the above-described additive for giving buffer action, for the convenience of preparing color developers, or for increasing the ionic strength.

The color developer may contain, if necessary, a development accelerator. For example, there are vari-

ous pyridinium compounds and other cationic compounds described in U.S. Pat. No. 2,648,604; Japanese Patent Publication 9503/69 and U.S. Pat. No. 3,671,247; cationic dyes such as phenosafranine; neutral salts such as thallium nitrate and potassium nitrate; nonionic compounds such as polythioethers, polyethylene glycol and the derivatives thereof described in Japanese patent publication No. 9504/69; and U.S. Pat. Nos. 2,533,990; 2,531,832; 2,950,970 and 2,577,127; the organic solvents and organic amines (e.g., ethanolamine, ethylenediamine, diethanolamine, etc.) described in Japanese patent publication 9509/69 and Belgian Patent 682,862 as well as the accelerators described in L. F. A. Mason, *Photographic Processing Chemistry*, pages 40-43 (Focal Press-London-1966). Also, benzyl alcohol and phenyl ethyl alcohol described in U.S. Pat. No. 2,515,147 and pyridine, ammonia, hydrazine, and amines described in *Journal of the Society of Photographic Science and Technology of Japan*; Vol. 14, pages 74 (1952) are also useful development accelerators.

Also, sulfites such as, for example, sodium sulfite, potassium sulfite, potassium hydrogensulfite, and sodium hydrogensulfite as well as hydroxylamine, ascorbic acid, pentose, hexose, etc., usually used as preservatives in photographic field may be added to the color 25 developers used in this invention.

Still further, the color developers used in this invention may further contain, if necessary, any desired anti-fogging agent. As the antifoggants used in this invention, there are alkali metal halides such as potassium bromide, sodium bromide, potassium iodide, etc., and organic antifoggants. Examples of organic antifoggants are nitrogen-containing heterocyclic compounds such as benzotriazole, 6-nitrobenzimidazole, 5-nitroisindazole, 5-methylbenzotriazole, 5-nitrobenzotriazole, 35 5-chlorobenzotriazole, etc.; mercapto-substituted heterocyclic compounds such as 1-phenyl-5-mercaptopentrazole, 2-mercaptopbenzimidazole, 2-mercaptopbenzothiazole, etc.; and mercapto-substituted aromatic compounds such as thiosalicylic acid, etc. Preferred examples of organic antifoggants are nitrogen-containing heterocyclic compounds, in particular nitrogen-containing heterocyclic compounds which have not been substituted by mercapto group. The proportion of the antifogging agent is about 1 mg to 5 g, preferably 5 mg to 1 g 40 45 per liter of the color developer.

Furthermore polyphosphoric acid compounds exemplified by sodium hexametaphosphate, sodium tetrapolyphosphate, sodium tripolyphosphate, potassium hexametaphosphate, potassium tetrapolyphosphate, potassium tripolyphosphate, etc.; or aminopolycarboxylic acids exemplified by phosphonocarboxylic acid,  $\alpha$ -aminoacid, ethylenediaminetetraacetic acid, nitrilotriacetic acid, cyclohexanediaminetetraacetic acid, iminodiacetic acid, N-hydroxymethylethylenediaminetriacetic acid, diethylenetriaminepentaacetic acid, etc., may be used as a water softener for the color developers. The addition amount of the material depends upon the hardness of water to be used but is usually about 0.5 to 1 g/liter.

Moreover, calcium or magnesium covering agents can be used in the photographic processing solutions in this invention. They are described in detail in, for example, J. Williams, *Belgische Chemische Industrie*, Vol. 21, page 325 (1956) and *ibid.*, Vol. 23, page 1105 (1958).

In the case of reversal color processing, competing couplers, fogging agents, and compensation developing agents may be used.

As the competing couplers, there are citrazinic acid, J-acid, H-acid, etc. Practical examples of these competing couplers used in this invention are described in U.S. Pat. No. 2,742,832; Japanese patent publications 9504/69; 9506/69 and 9507/69 and U.S. Pat. Nos. 3,520,690; 3,560,212; 3,645,737; etc.

As the fogging agents used in this invention, there are alkali metal borohydrides (e.g., sodium borohydride), amineboranes (e.g., t-butylamineborane), tin-aminopolycarboxylic acid complex salts, tin-pyrophosphoric acid complex salts, tin-tetrapolyphosphoric acid complex salts, tin-hexametaphosphoric acid complex salts, ethylenediamine, etc. Also, the compounds described in Japanese patent publication 38816/72 are useful for the fogging agent.

As the compensation developing agents used in this invention, there are p-aminophenyl, N-benzyl-p-aminophenol, 1-phenyl-3-pyrazolidone, etc. Other examples of the compensation developing agent used advantageously in this invention are described in, for example, Japanese patent publications Nos. 41475/70 and 19037/71.

The pH of the color developer used in this invention is about 7 to 14, preferably about 8 to 13.

The processing process of this invention can be applied not only to a color photographic system wherein dye forming couplers are incorporated in color photographic materials as described in, for example, U.S. Pat. Nos. 2,322,027; 2,376,679 and 2,801,171 but also to a color photographic system wherein couplers are incorporated in color developers as described in, for example, U.S. Pat. Nos. 2,252,718; 2,590,970 and 2,592,243.

At present, however, the former system is mainly performed. In the case that dye forming couplers are incorporated in color photographic materials, multi-layer color photographic materials are generally used and in this case it is preferred that the couplers remain in definite emulsion layers and do not diffuse into other emulsion layers during the production steps thereof, preservation, and processing steps for them.

A fix solution having a composition usually used for the purpose can be used in this invention. As a fixing agent, there are thiosulfates, thiocyanates, thioureas, thioglycols, water-soluble organic diols containing sulfur or oxygen in the molecule (e.g., 3,6-dithia-1,8-octyl-diol), etc. The fixing solution may further contain a stabilizer such as a sulfite (e.g., sodium sulfite), etc., and a pH buffering salt or a swelling inhibiting salt (e.g., a hardening agent such as potassium alum) and when a thiosulfate is used as the fixing agent, the use of the aforesaid stabilizer is particularly preferred.

Moreover, the black and white developer used in a silver dye bleaching process or a reversal color photographic process in this invention may contain a developing agent generally used in black and white developers. As the developing agent, a dihydroxybenzene (e.g., hydroquinone, sodium hydroquinonemonosulfonate, etc.), a 3-pyrazolidone (e.g., 1-phenyl-3-pyrazolidone, etc.), an aminophenol (e.g., N-methyl-p-aminophenol, etc.), ascorbic acid, etc., may be used solely or as a combination thereof. The developer may further contain a preservative, an alkalinizing agent, a pH buffer, an antifogging agent, etc., and also, if necessary, it may further contain a dissolution aid, a toning agent, a development accelerator, a surface active agent, a defoaming agent, a water softener, a hardening agent, a tackifier, etc., well-known about the detail of them in the field of the art.

The photographic silver halide emulsion layers of the color photographic materials used in this invention may contain color image-forming couplers, that is, the compounds forming dyes by the reaction with the oxidation product of an aromatic amine (usually primary amine) developing agent (hereinafter, referred to as simply couplers). The couplers are preferably non-diffusible ones having a hydrophobic group called as a ballast group in the molecule. The couplers may be 4-equivalent ones or two-equivalent ones for silver ion. Also, the silver halide emulsion layers may further contain colored couplers having an effect of color correction or couplers releasing a development inhibitor with the progress of development (i.e., so-called DIR couplers). Still further, the couplers may be couplers providing colorless products by the coupling reaction thereof.

As a yellow coupling coupler, known open chain ketomethylene couplers can be used. In particular, benzoylacetanilide series compounds and pivaloylacetanilide series compounds are advantageously used in this invention. Practical examples of the yellow coupling couplers are described in U.S. Pat. Nos. 2,875,057; 3,265,506; 3,408,194; 3,551,155; 3,582,322; 3,725,072; and 3,891,445; West German patent No. 1,547,868; West German patent publications (OLS) Nos. 2,219,917; 2,261,361 and 2,414,006; U.K. Pat. No. 1,425,020; Japanese patent publication No. 10783/76; and Japanese patent applications (OPI) Nos. 26133/72; 73147/73; 102636/76; 6341/75; 123342/75; 130442/75; 21827/76; 87650/75; 82424/77 and 115219/77.

As the magenta coupling couplers used in this invention, there are pyrazolone series compounds, indazolone series compounds, and cyanoacetyl series compounds but in particular, pyrazolone series compounds are more useful. Practical examples of the magenta coupling couplers are described in U.S. Pat. Nos. 2,600,788; 2,983,608; 3,062,653; 3,127,269; 3,311,476; 3,419,391; 3,519,429; 3,558,319; 3,582,322; 3,615,506; 3,834,908; and 3,891,445; West German Pat. No. 1,810,464; West German patent application (OLS) Nos. 2,408,665; 2,417,945; 2,418,959 and 2,424,467; Japanese patent publication Nos. 6031/65 and 45990/76; and Japanese patent application (OPI) Nos. 20826/76; 58922/77; 129538/74; 74027/74; 159336/75; 42121/77; 74028/74; 60233/75; 26541/76 and 55122/78.

As the cyan coupling couplers used in this invention, there are phenol series compounds, naphthol series compounds, etc. Practical examples of them are described in U.S. Pat. Nos. 2,369,929; 2,434,272; 2,474,293; 2,521,908; 2,895,826; 3,034,892; 3,311,476; 3,458,315; 3,476,563; 3,583,971; 3,591,383; 3,767,411 and 4,004,929; West German patent application (OLS) Nos. 2,414,830 and 2,454,329; and Japanese patent application (OPI) Nos. 59838/73; 26034/76; 5055/73; 146828/76; 69624/77 and 90932/77.

Examples of the colored couplers used in this invention are described in, for example, U.S. Pat. Nos. 3,476,560; 2,521,908 and 3,034,892; Japanese patent Publication Nos. 2016/69; 22335/63; 11304/67 and 32461/69; Japanese patent application (OPI) Nos. 26034/76 and 42121/77 and West German patent application (OLS) No. 2,418,959.

Also, examples of the DIR couplers used in this invention are described in, for example, U.S. Pat. Nos. 3,227,554; 3,617,291; 3,701,783; 3,790,384 and 3,632,345; West German patent application (OLS) Nos. 2,414,006; 2,454,301 and 2,454,329; U. K. Pat. Nos. 953,454; Japanese patent application (OPI) Nos. 69624/77; 122335/74

and 69624/77 and Japanese patent publication No. 16141/76.

The color photographic materials used in this invention may further contain compounds releasing a development inhibitor at development and examples of these compounds are described in, for example, U.S. Pat. Nos. 3,297,445 and 3,379,529; West German patent application (OLS) No. 2,417,914; and Japanese patent application (OPI) Nos. 15271/77 and 9116/78.

The couplers described above may be incorporated as a combination of two or more couplers in the same silver halide emulsion layer of a color photographic material or the same coupler may be incorporated in two or more silver halide emulsion layers of a color photographic material.

These couplers are dispersed in silver halide photographic emulsions together with a solvent having a proper polarity. Useful solvents for the purpose are tri-o-cresyl phosphate, trihexyl phosphate, dioctylbutyl phthalate, dibutyl phthalate, diethyl lauryl amide, 2,4-diallyl phenol, octyl benzoate, etc.

Typical examples of the color image forming materials used in the color photographic materials for silver dye bleach process processed according to this invention are, for example, azo dyes.

The color photographic material processed according to this invention has at least one silver halide emulsion layer on a support and usually has a red sensitive silver halide emulsion layer, a green sensitive silver

halide emulsion layer and a blue sensitive silver halide emulsion layer on a support. More practically, the color photographic material used in this invention has usually at least a red sensitive silver halide emulsion layer containing a cyan image forming coupler, at least a green sensitive silver halide emulsion layer containing a magenta image forming coupler, and at least a blue sensitive silver halide emulsion layer containing a yellow image forming coupler. Such a color photographic element may further include non-photosensitive photographic layers (e.g., antihalation layer, interlayer for color mixing prevention, etc., yellow filter layer, protective layer, etc.). Also, there is no particular restriction about the order of the red sensitive emulsion layer, the green sensitive emulsion layer and the blue sensitive emulsion layer described above. The silver halide photographic emulsions used in this invention may be surface latent image type emulsions or inside latent image type emulsions which are prepared by known processes.

As described above in detail, there are no particular restrictions on the process for producing the silver halide emulsions of color photographic materials used in this invention, the layer structures of the color photographic materials, photographic additives, photographic elements, and photographic processing solutions.

By employing the bleach composition of this invention, the following advantages are obtained:

- (1) Environmental pollution is reduced.
- (2) Bleaching speed is high.
- (3) Stains do not occur.
- (4) So-called inferior recoloring in which dyes formed in a development step remain as leuco dyes even after the bleaching step does not occur.
- (5) The reduction in bleaching faculty when the bleach solution is allowed to stand for a long period of time is less and hence the bleach solution can be stably stored for a long period of time.

(6) The bleach solution can be easily regenerated for reuse.

The invention will now be further explained in the following example.

### EXAMPLE

A color reversal photographic material was prepared by coating a triacetate film successively with the following layers in order.

1st layer (red sensitive silver halide emulsion layer):

The coating composition for the emulsion layer was prepared by mixing a red sensitive silver iodobromide emulsion (silver iodide: 7 mole percent) and a cyan coupler emulsion (containing 1-hydroxy-4-chloro-2-n-dodecylnapthamide as a cyan coupler and dibutyl phthalate as a coupler solvent) in such a manner that the silver/coupler mole ratio became 8.0. The coverage of silver was 1.5 g/m<sup>2</sup>.

2nd layer (intermediate layer):

A gelatin intermediate layer containing di-t-amyl hydroquinone dispersed therein.

3rd layer (green sensitive silver halide emulsion layer):

The coating composition for the emulsion layer was prepared by mixing a green sensitive silver iodobromide emulsion (silver iodide: 6 mole percent) and a magenta coupler emulsion (containing 1-(2,4,6-trichlorophenyl)-3-[3-(2,6-di-t-amylphenoxyacetamido)benzamido]-5-pyrazolone as a magenta coupler and tricresyl phosphate as a coupler solvent) in such a manner that the silver/coupler mole ratio became 9.5. The coverage of silver: 1.5 g/m<sup>2</sup>.

4th layer (yellow filter layer):

A filter layer composed of yellow colloid silver and gelatin.

5th layer (blue sensitive silver halide emulsion layer):

The coating composition for the emulsion layer was prepared by mixing a blue sensitive silver iodobromide emulsion (silver iodide: 6 mole percent) and a yellow coupler emulsion (containing  $\alpha$ -pivaloyl-2-chloro-5-[ $\gamma$ -(2,4-di-t-amylphenoxy)butanamido]acetanilide as a yellow coupler and dibutyl phthalate as a coupler solvent) in such a manner that the silver/coupler mole ratio became 8.0. The coverage of silver: 1.8 g/m<sup>2</sup>.

The 6th layer (protective layer):

A protective layer mainly composed of gelatin.

The color reversal photographic film was exposed through an optical wedge to a tungsten lamp as a light source for 1/100 sec., and thereafter subjected to the following reversal processings:

| Processing step                   | Temperature | Time           |
|-----------------------------------|-------------|----------------|
| 1st Development (black and white) | 43° C.      | 2 min.         |
| Stop                              | 40° C.      | 20 sec.        |
| Wash                              | 40° C.      | 40 sec.        |
| Color Development                 | 46° C.      | 2 min.         |
| Stop                              | 40° C.      | 20 sec.        |
| Wash                              | 40° C.      | 1 min.         |
| Bleach                            | 40° C.      | 1 min. 30 sec. |
| Fix                               | 40° C.      | 40 sec.        |
| Wash                              | 40° C.      | 1 min.         |
| Stabilization                     | 40° C.      | 20 sec.        |
| Dry                               | 37° C.      |                |

The compositions of the processing solutions used in the above processing steps were as follows:

#### The 1st Developer:

Sodium Sulfite 60.0 g

-continued

|    |                                                                               |            |
|----|-------------------------------------------------------------------------------|------------|
| 1  | 1-Phenyl-3-pyrazolidone                                                       | 0.3 g      |
|    | Hydroquinone                                                                  | 5.0 g      |
|    | Sodium Carbonate (monohydrate)                                                | 41.0 g     |
|    | Potassium Bromide                                                             | 2.0 g      |
|    | Potassium Iodide (1% aq. soln.)                                               | 1.0 ml     |
|    | Potassium Thiocyanate (1N aq. soln.)                                          | 10.0 ml    |
|    | Sodium hydroxide (10% aq. soln.)                                              | 2.0 ml     |
|    | Water to make                                                                 | 1.0 liter. |
|    | <u>Stop Solution:</u>                                                         |            |
| 10 | Sodium Acetate                                                                | 30 g       |
|    | Glacial Acetic Acid                                                           | 8 ml       |
|    | Water to make                                                                 | 1 liter.   |
|    | <u>Color Developer:</u>                                                       |            |
|    | Benzyl Alcohol                                                                | 5.0 ml     |
|    | Sodium Hydroxide                                                              | 0.5 g      |
|    | Diethylene Glycol                                                             | 3.0 ml     |
|    | Sodium Hexametaphosphate                                                      | 2.0 g      |
|    | Sodium Sulfite                                                                | 2.0 g      |
|    | Potassium Bromide                                                             | 2.0 g      |
|    | Ethyl-N-( $\beta$ -methanesulfonamido-ethyl)aniline sesquisulfate monohydrate | 9.0 g      |
|    | Citrazinic Acid                                                               | 0.4 g      |
|    | Metaboric Acid                                                                | 0.5 g      |
|    | Sodium Metaborate tetrahydrate                                                | 77.0 g     |
|    | Sodium Borohydride                                                            | 0.1 g      |
|    | Water to make                                                                 | 1 liter.   |
|    | <u>Bleach Solution:</u>                                                       |            |
|    | Bleach Solution-1:                                                            |            |
|    | Potassium Ferricyanide                                                        | 50 g       |
|    | Potassium Bromide                                                             | 25 g       |
|    | Sodium Primary Phosphate                                                      | 1 g        |
|    | Water to make                                                                 | 1 liter.   |
|    | <u>Fix Solution:</u>                                                          |            |
|    | Sodium Thiosulfate                                                            | 200 g      |
|    | Sodium Sulfite                                                                | 15 g       |
|    | Borax                                                                         | 12 g       |
|    | Glacial Acetic Acid                                                           | 15 ml      |
|    | Water to make                                                                 | 1 liter.   |
|    | <u>Stabilizing Solution:</u>                                                  |            |
|    | Formalin (37%)                                                                | 10 ml      |
|    | Fuji Dry Well (trade name, made by Fuji Photo Film Co.)                       | 5 ml       |
|    | Water to make                                                                 | 1 liter.   |

The same procedure as above was followed by changing the bleaching time and the composition for the bleach solution as follows:

Bleaching Time: 1 min., 2 min., 2 min. 30 sec., 3 min., 45 3 min. 30 sec., 5 min., 10 min., 20 min.

|    |                                   |          |
|----|-----------------------------------|----------|
| 50 | <u>Bleach Solution:</u>           |          |
|    | Bleach Solution-2:                |          |
|    | Ethylenediaminetetraacetic Acid   | 0.5 g    |
|    | 2-sodium Salt                     |          |
|    | Ethylenediaminetetraacetic Acid   |          |
|    | Ferric Ammonium Dihydrate         | 10 g     |
|    | Ammonium Bromide                  | 100 g    |
|    | Acetic Acid                       | 20 ml    |
|    | Aqueous ammonia and water to make | 1 liter. |
|    | pH                                | 4.0      |
|    | <u>Bleach Solution-3:</u>         |          |
|    | Ammonium Bromide                  | 100 g    |
|    | Acetic Acid                       | 20 ml    |
|    | 30% Hydrogen Peroxide             | 50 ml    |
|    | Aqueous ammonia and water to make | 1 liter. |
|    | pH                                | 4.0      |
|    | <u>Bleach Solution-4:</u>         |          |
|    | Ethylenediaminetetraacetic Acid   | 0.5 g    |
|    | 2-sodium Salt                     |          |
|    | Ethylenediaminetetraacetic Acid   |          |
|    | Ferric Ammonium Dihydrate         | 10 g     |
|    | Ammonium Bromide                  | 100 g    |
|    | Acetic Acid                       | 20 ml    |
|    | 30% Hydrogen Peroxide             | 50 ml    |
|    | Aqueous ammonia and water to make | 1 liter. |

-continued

Bleach Solution:

### Bleach Solution-5:

To 1 liter of Bleach Solution-4 was added 2 g of the monohydrate of Compound (1) illustrated before and the pH of the solution was adjusted to 4.0.

### Bleach Solution-6:

To 1 liter of Bleach Solution-4 was added 2 g of the di-sodium salt of Compound (12) and the pH of the solution was adjusted to 4.0.

### Bleach Solution-7:

To 1 liter of Bleach Solution-4 was added 2 g of Compound (18) and the pH of the solution was adjusted to 4.0.

### Bleach Solution-8:

To 1 liter of Bleach Solution-4 was added 2 g of Compound (21) and the pH of the solution was adjusted to 4.0.

### Bleach Solution-9:

To 1 liter of Bleach Solution-4 was added 2 g of Compound (25) and the pH of the solution was adjusted to 4.0.

|                                   |          |
|-----------------------------------|----------|
| Bleach Solution-10:               |          |
| Ethylenediaminetetraacetic Acid   |          |
| 2-sodium Salt                     | 0.5 g    |
| Ethylenediaminetetraacetic Acid   |          |
| Ferric Ammonium Dihydrate         | 4 g      |
| Ammonium Bromide                  | 100 g    |
| Acetic Acid                       | 20 ml    |
| 30% Hydrogen Peroxide             | 50 ml    |
| Aqueous ammonia and water to make | 1 liter. |
| pH                                | 4.0      |

### Bleach Solution-11:

To 1 liter of Bleach Solution-10 was added 2 g of Compound (25) and the pH was adjusted to 4.0.

The periods of time required for bleaching (the time when the total remained amount of silver in the color photographic film bleached became almost same as the total remaining amount of silver in the color photographic film bleached by Bleach Solution-1 (bleaching time: 1 min. 30 sec.) are shown in the following table as the photographic properties obtained by the processings using Bleach Solutions 2-11.

Furthermore, for determining the storage stability of a part of the bleach solutions, each of the bleach solutions was allowed to stand for 5 days at 20° C. or for 4 days at 40° C. and then the residual percentage of hydrogen peroxide in the bleach solution was measured, the results being also shown in the same table.

TABLE

| Bleach<br>Solution | Time required<br>to Finish<br>Bleaching | Storage<br>Stability<br>(residual %<br>of $H_2O_2$ ) |                         |   | Remarks    |
|--------------------|-----------------------------------------|------------------------------------------------------|-------------------------|---|------------|
|                    |                                         | 20° C.<br>for<br>5 days                              | 40° C.<br>for<br>4 days |   |            |
| Solution-1         | 1 min. 30 sec.                          | —                                                    | —                       | — | Comparison |
| Solution-2         | 20 min.                                 | —                                                    | —                       | — | Comparison |
| Solution-3         | scarcely<br>bleached                    | 90%                                                  | 60%                     | — | Comparison |
| Solution-4         | 2 min. 30 sec.                          | 40%                                                  | 0.1%                    | — | Comparison |
| Solution-5         | 2 min. 30 sec.                          | 80%                                                  | —                       | — | Invention  |
| Solution-6         | 2 min. 30 sec.                          | 70%                                                  | —                       | — | Invention  |

TABLE-continued

| 5  | Bleach<br>Solution | Time required<br>to Finish<br>Bleaching | Storage<br>Stability<br>(residual %<br>of $H_2O_2$ ) |                         |            |
|----|--------------------|-----------------------------------------|------------------------------------------------------|-------------------------|------------|
|    |                    |                                         | 20° C.<br>for<br>5 days                              | 40° C.<br>for<br>4 days | Remarks    |
| 10 | Solution-7         | 2 min. 30 sec.                          | 83%                                                  | 50%                     | Invention  |
|    | Solution-8         | 2 min. 30 sec.                          | 80%                                                  | —                       | Invention  |
|    | Solution-9         | 2 min. 30 sec.                          | 88%                                                  | 54%                     | Invention  |
|    | Solution-10        | 3 min.                                  | 55%                                                  | 0.3%                    | Comparison |
|    | Solution-11        | 3 min.                                  | 90%                                                  | 60%                     | Invention  |

From the results shown in the above table, it will be understood that the bleach solutions of this invention had excellent storage stability and the addition of the compound having a sulfon group did not give any influences on the time required for finishing the bleach and the bleach solutions of this invention showed high bleaching speed even by the addition of such a compound.

While the invention has been described in detail and with reference to specific embodiments thereof, it will be apparent to one skilled in the art that various changes and modifications can be made therein without departing from the spirit and scope thereof.

What is claimed is:

1. A bleach solution for silver halide color photographic materials comprising hydrogen peroxide and/or a compound releasing hydrogen peroxide, an organic metal complex salt which is a chelate of a polycarboxylic acid represented by formula (I), an aminopolycarboxylic acid represented by formula (II) or an organic phosphonic acid represented by formula (III-a) or (III-b) and a high valent metal ion,



wherein  $R_1$  represents a single bond, an unsubstituted or substituted alkylene group having 1 to 6 carbon atoms wherein the substituent is a hydroxy group and/or a carboxy group, a  $-(CH_2)_m-O-(CH_2)_n-$  group wherein  $m$  and  $n$  are integers and  $m+n$  is 2 to 6, a  $-(CH_2)_m-S-(CH_2)_n-$  group wherein  $m'$  and  $n'$  are integers and  $m'+n'$  is 2 to 6, or an alkenylene group having 2 to 6 carbon atoms;  $l$  represents an integer of 2 to 3; and when  $R_1$  is a single bond,  $l$  is 2,



55 wherein R<sub>2</sub>, R<sub>3</sub>, R<sub>4</sub> and R<sub>5</sub> each represents a carboxyalkyl group wherein the alkyl moiety has 1 to 2 carbon atoms, a hydroxylalkyl group having 1 to 2 carbon atoms and/or a hydrogen atom; p represents zero or an integer of 1 to 3; L represents an alkylene group having 2 to 4 carbon atoms, a  $-\text{CH}_2\text{x}[\text{O}-(\text{CH}_2\text{y})\text{z}]$  group 60 wherein x is an integer of 2 to 4, y is an integer of 2 to 4 and z is an integer of 1 to 3, a 6-membered cyclic alkylene group, or an arylene group; and the aminopolycarboxylic acid of the formula (II) has at least 65 1 carboxy group,



wherein  $R_6$  represents a substituted or unsubstituted alkyl or alkylene group having 1 to 4 carbon atoms wherein the substituent is a hydroxy group and/or a carboxy group, or a substituted or unsubstituted diaminoalkylene group having 2 to 16 carbon atoms wherein the substituent is a hydroxy group;  $L$  represents an alkylene group having 1 to 2 carbon atoms; and  $q$  represents an integer of 1 to 5, and at least one aromatic sulfonic acid or salt or salt thereof, said aromatic sulfonic acid or salt thereof being present in an concentration of  $10^{-3}$  to 0.1 mole per liter of bleaching solution, said bleach solution having a pH of about 1 to 8.

2. The bleach solution of claim 1, wherein said high valent metal ion is of iron, cobalt, or copper.

3. The bleach solution of claim 1, wherein said metal ion is a ferric ion.

4. The bleach solution of claim 1, wherein hydrogen peroxide or a compound capable of releasing hydrogen peroxide is present in an amount of about 0.01 to 10 mols per liter of bleach solution.

5. The bleach solution of claim 1, wherein said aromatic sulfonic acid is represented by the formula (III)



(III)

wherein  $M$  represents a hydrogen atom, an alkali metal atom, or an ammonium group;  $r$  represents an integer of 1 to 5 and  $Q$  represents an aromatic hydrocarbon group or an aromatic heterocyclic group including at least one nitrogen atom or sulfur atom.

6. The bleach solution of claim 5, wherein said aromatic group may be substituted by one or more substituents selected from the group consisting of aliphatic and aromatic hydrocarbon groups, a carboxy group, a hydroxy group, an amino group, a nitro group, a nitroso group or a halogen atom.

7. The bleach solution of claim 1, which additionally comprises an alkali or an ammonium halide.

8. The bleach solution of claim 1, which additionally comprises an aliphatic carboxylic acid, an aliphatic sulfonic acid, or an aliphatic phosphonocarboxylic acid.

9. In a process for developing a color photographic material including a bleaching step, the improvement which comprises bleaching said material in a solution containing hydrogen peroxide and/or a compound capable of releasing hydrogen peroxide, an organic metal complex salt which is a chelate of an aminopolycarboxylic acid, an organic phosphonic acid, or a polybasic organic acid and a high valent metal ion, and at least one aromatic sulfonic acid or salt thereof, said aromatic sulfonic acid or salt thereof being present in a concentration of  $10^{-3}$  to 0.1 mole per liter of bleaching solution.

10. The process of claim 9, wherein said high valent metal ion is of iron(III), cobalt(III), or copper(II).

11. The process of claim 9, wherein said chelating agent is represented by formula (I), (II), (III-a) or (III-b):



(I)

ps wherein  $R_1$  represents a single bond, an unsubstituted or substituted alkylene group having 1 to 6 carbon atoms wherein the substituent is a hydroxy group and/or a carboxy group, a  $-(CH_2)_m-O-(CH_2)_n-$  group wherein  $m$  and  $n$  are integers and  $m+n$  is 2 to 6, a  $-(CH_2)_m'-S-(CH_2)_n'-$  group wherein  $m'$  and  $n'$  are integers and  $m'+n'$  is 2 to 6, or an alkenylene group

10 25 wherein  $R_6$  represents a substituted or unsubstituted alkyl or alkylene group having 1 to 4 carbon atoms wherein the substituent is a hydroxy group and/or a carboxy group, or a substituted or unsubstituted diaminoalkylene group having 2 to 16 carbon atoms wherein the substituent is a hydroxy group;  $L$  represents an alkylene group having 1 to 2 carbon atoms; and  $q$  represents an integer of 1 to 5.

12. The process of claim 9, wherein said metal ion is a ferric ion.

13. The process of claim 9, wherein hydrogen peroxide or a compound capable of releasing hydrogen peroxide is present in an amount of about 0.01 to 10 mols per liter of bleach solution.

14. The process of claim 9, wherein said aromatic sulfonic acid is represented by the formula (III):



(III)

45 wherein  $M$  represents a hydrogen atom, an alkali metal atom, or an ammonium group;  $r$  represents an integer of 1 to 5 and  $Q$  represents an aromatic hydrocarbon group or an aromatic heterocyclic group including at least one nitrogen atom or sulfur atom.

15. The process of claim 14, wherein said aromatic group may be substituted by one or more substituents selected from the group consisting of aliphatic and aromatic hydrocarbon groups, a carboxy group, a hydroxy group, an amino group, a nitro group, a nitroso group, or a halogen atom.

16. The process of claim 9 which additionally comprises an alkali or an ammonium halide.

17. The process of claim 9, which additionally comprises an aliphatic carboxylic acid, an aliphatic sulfonic acid, or an aliphatic phosphonocarboxylic acid.

18. The process of claim 9, wherein said composition provides a bleach solution having a pH of about 1 to 10.

19. The process of claim 9, wherein prior to bleaching with said solution, said photograph material is bleached with a solution containing a substituted alkylthiol compound or a precursor thereof.

20. The process of claim 19, wherein said alkylthiol compound is represented by the formula

having 2 to 6 carbon atoms;  $l$  represents an integer of 2 to 3; and when  $R_1$  is a single bond,  $l$  is 2,



10 15 wherein  $R_2$ ,  $R_3$ ,  $R_4$  and  $R_5$  each represents a carboxyalkyl group wherein the alkyl moiety has 1 to 2 carbon atoms, a hydroxyalkyl group having 1 to 2 carbon atoms and/or a hydrogen atom;  $p$  represents zero or an integer of 1 to 3;  $L$  represents an alkylene group having 2 to 4 carbon atoms, a  $-(CH_2)_x[O-(CH_2)_y]_z-$  group wherein  $x$  is an integer of 2 to 4,  $y$  is an integer of 2 to 4 and  $z$  is an integer of 1 to 3, a 6 membered cyclic alkylene group, or an arylene group; and the aminopolycarboxylic acid of the formula (II) has at least 1 carboxy group,



25 30 wherein  $R_6$  represents a substituted or unsubstituted alkyl or alkylene group having 1 to 4 carbon atoms wherein the substituent is a hydroxy group and/or a carboxy group, or a substituted or unsubstituted diaminoalkylene group having 2 to 16 carbon atoms wherein the substituent is a hydroxy group;  $L$  represents an alkylene group having 1 to 2 carbon atoms; and  $q$  represents an integer of 1 to 5.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350

R—S—Y

wherein R represents an alkyl group containing 1 to 10 carbon atoms, which may be substituted with one or more substituents selected from the group consisting of a hydroxy group, a primary, a secondary, or a tertiary amino group, a carboxy group, a sulfon group, a piperidino group, a pyrrolyl group, a morpholino group, an

imidazole group, and a benzotriazole group; and Y represents a hydrogen atom or an amidino group.

21. The process of claim 9, wherein said process is a direct color process.

5 22. The process of claim 9, wherein said process is a color reversal process.

23. The process of claim 18, wherein the pH is about 1 to 8.

\* \* \* \* \*

10

15

20

25

30

35

40

45

50

55

60

65